

## UNITED STATES PATENT OFFICE

1,957,474

## PAPER MANUFACTURE

Harold Robert Rafton, Andover, Mass., assignor  
to Raffold Process Corporation, a corporation  
of Massachusetts

No Drawing. Application July 8, 1932,  
Serial No. 621,509

26 Claims. (Cl. 92—21)

This invention relates to the manufacture of paper filled with alkaline filler.

The principal object of this invention is the employment in the manufacture of paper filled with alkaline filler of substantially water insoluble organic material of a non-waxy nature substantially inert to alkaline filler, said material being either of a pasty or liquid consistency.

An important object is the use of such material to modify the characteristics of the paper in the manufacture of which it is employed.

A further object is the use of such material to produce a sized paper filled with alkaline filler.

A further object is to produce alkaline filled paper of especially high receptivity to printing ink.

Other objects and advantages of the invention will become apparent during the course of the following description.

20 In my Patent No. 1,819,441, granted August 18, 1931, I disclose paper filled with alkaline filler and sized with waxy substantially water insoluble material substantially inert to alkaline filler, such for example as paraffin or other hydrocarbon. I 25 state that the paraffin employed may be of high or low melting point and that it may be fully refined or may contain impurities, such for example as oil.

While at room temperature fully refined paraffin is a waxy solid, it will be apparent that the presence of pasty or liquid impurities, usually hydrocarbons, will produce an admixture of modified characteristics which may vary by imperceptible degrees from the waxy solid of fully refined paraffin through various pasty consistencies from a stiff paste to a softer paste and even down to a liquid, depending upon the kind and amount of impurities admixed with the paraffin.

In accordance with the disclosure in my above referred to patent wherein, as stated, the use of impure as well as of pure waxy material is described, such admixtures have been found to give a measure of sizing, the degree of which has been found in certain cases to be roughly proportional 45 to the amount of waxy material present.

Thus, where waxy material as above has been employed in admixture with impurities it was believed that the waxy material alone was substantially responsible for the sizing effect imparted, and that the accompanying materials acting as impurities were substantially without sizing or other beneficial effect.

I have found however that under certain conditions it is possible to attain a moderate degree 50 of success in sizing paper filled with alkaline

filler if, instead of using the above described waxy materials or mixtures of these with substantially water insoluble non-waxy material substantially inert to alkaline filler which give a resultant admixture of pasty or even liquid consistency, I employ by itself organic substantially water insoluble non-waxy material substantially inert to alkaline filler, which may vary from a pasty consistency by imperceptible steps down to the liquid condition. I have found that such non-waxy material will 60 in itself impart a certain degree of sizing to paper filled with alkaline filler in the absence of any appreciable or substantial amount of waxy material such as is described in my above referred to patent, and where in the claims appended hereto I speak of non-waxy material or the like "in the absence of" waxy material or the like, I intend the phrase "in the absence of" to mean "in the absence of any substantial amount of." I have found however that, for purposes of sizing, 75 such non-waxy material of liquid consistency does not appear to be so effective as such material of pasty consistency, and of the pasty materials the stiffer pasty ones are more effective than the softer pasty ones, but in general even the stiffer 80 pasty ones are not so effective as the waxy materials previously disclosed.

However, this relative inefficiency of sizing quality compared with waxy material may be overcome in certain cases by the use of larger 85 quantities of the non-waxy material in question, and in certain instances the cost of such material in comparison with the cost of waxy material makes it feasible and sometimes economical to use such non-waxy material. Furthermore, 90 such non-waxy material may also in certain cases be used advantageously where only a small degree of sizing, say only from one to a few seconds sizing test (as tested by flotation on aqueous ink), is desired to be imparted to the resulting paper. 95 Also, its use seems to be advantageous in certain cases where practically no so-called sizing test is wanted but where an enhanced receptivity to printing ink is desired to be imparted, which such material seems to possess the ability to impart. 100 This is a characteristic of importance in paper to be used for printing and particularly for color work on high speed presses. Paper made according to the present invention appears to possess such greater receptivity to printing ink and thus 105 to produce clearer impressions with less tendency to offset than the alkaline filled papers hitherto made, excepting perhaps those made with waxy material according to my prior process.

My invention may be summarized as the process 110

of including organic substantially water insoluble non-waxy material substantially inert to alkaline filler, of either pasty or liquid consistency, in paper filled with alkaline filler to impart to the paper so made certain characteristics, such as sizing of varying degree as desired, or greater printing ink receptivity with freedom from offset, or the like. Of course, it will be understood that the conjoint use in paper of such material with any substantial amount of waxy material is not novel because of the disclosure in my prior patent above referred to.

In the practice of my invention I may proceed by either of two modifications. I may either incorporate the non-waxy material into the paper mix before web formation or in the web during web formation, or I may apply it to the paper web subsequent to web formation.

According to the first modification I may introduce in the beater (or other mixing device) with fibrous material and alkaline filler the non-waxy material, preferably in emulsion form. The order of addition may be varied as desired. I may run this mix off on the paper machine with satisfactory results, but in general I prefer to employ a precipitant for the emulsion, such as an acidic material, for example, alum.

With certain types of emulsions such as the substantially non-breakable or insoluble emulsifier type, I may dispense with a precipitant, as above, or may use an acidic material or metallic salt such as alum; but with this type of emulsion I sometimes find it convenient to employ two mutually precipitable materials such as rosin size and alum, or sodium silicate and acidic material, or the like, which act to concentrate the disperse phase of the emulsion upon the fibre. Such mutually precipitating materials may also be used with other types of emulsions if desired.

I may, generally with improved results, employ the "minimizing principle" in connection with the first modification of my invention. This principle has been described in a number of my issued patents, and in its practical application consists briefly in substantially avoiding or minimizing the effect of alkaline filler on acidic material by adding one or more of the papermaking ingredients, such as alkaline filler, acidic material, material affected by alkaline filler, and the like, to the mix under conditions favoring the minimizing of the time and/or intimacy of contact of the constituents of the mix, e. g. at or subsequent to the point where the fibrous mix is about to leave the last chest in the stock system, commonly known as the machine chest, and prior to the point of delivery of the mix to the web-forming device. While the material may as stated be added at any point between the two indicated, I prefer to add the material at the mixing box, or at any point between the mixing box and the web-forming device, i. e. at the dilute stage of the papermaking operation.

The non-waxy material need not be added independently to the mix. It may be premixed with one or more of the other ingredients, e. g. alkaline filler, or with part or all of the fibre, or with acidic material such as alum, in the presence of a colloid such as starch or colloidal clay, if desired, and while such premixed ingredients may be added in the beater or other point in the stock system, it is especially advantageous in certain cases to add them under conditions favoring the minimizing of the time and/or intimacy of contact of the constituents of the mix as described in detail above.

I have stated above that I preferably employ the non-waxy material in emulsion form. While emulsions are my preferred method of employment they are not always necessary, as sometimes adequate incorporation of the non-waxy material in the mix may be attained by intimate mixing with one or more of the ingredients of the mix without prior emulsification, or even in special cases by direct addition to the mix itself, either in the beater or later if desired. In such cases elevated temperature in the stock is advantageous if non-waxy material of pasty consistency be used.

If an emulsion be used I may prepare such an emulsion in a variety of known ways, a number of methods of preparing emulsions being described in my already issued patents. For example, I may use as an emulsifying agent a saponified material such as a soap, for example ammonium oleate, or stearate, or rosin size, or the like, said saponified material either being used as such or formed during emulsification; or gums such as gum ghatti, with dextrin if desired; or insoluble emulsifying agents such as clay, preferably colloidal clay, or two mutually precipitable materials producing an insoluble agent; or casein solution, sodium silicate, or the like. Such methods of emulsification and others, as well as means for effecting them, are known in the art and are sufficiently familiar or so readily available to the chemist, that further description is here unnecessary.

It is to be understood of course that there may be used conjointly in the manufacture of papers so made, other sizing or treating agents, such as rosin size and the like, either directly with the non-waxy material, or added separately. Starch is especially useful in this connection.

As stated above, in this first modification of my invention I may if desired add the non-waxy material to the forming web on the web-forming device. The discussion above relative to condition in which the material is added, and ingredients added in connection therewith applies here with equal force. The application of the material is in general more difficult at this point insofar as a Fourdrinier machine is concerned, owing to possible interference with sheet formation, but this difficulty is not so manifest with a cylinder machine. However, in general I prefer the addition to the fibrous mix rather than during web formation.

In the second modification of my invention I apply the non-waxy material to the already formed web either on the paper machine or later. For this purpose I may employ an emulsion of the non-waxy material, with or without a precipitant, but I prefer a solution in an organic solvent, using if desired methods of application similar to those described in detail in my copending applications Serial No. 487,377, filed October 8, 1930, and Serial No. 609,555, filed May 5, 1932. Such methods comprise briefly the application to the paper web, either on the paper machine or later, of the non-waxy material, preferably in solution form, by spray, trough, contact roll or the like, and in the case where a solution in an organic solvent is used the subsequent removal of the solvent by evaporation, suitably by heat (which may in certain cases if desired be sufficient only substantially to supply the latent heat of evaporation of the solvent) or reduced pressure or both. In the interest of economy suitable means for recovery of solvent may be provided.

If the solvent used is non-miscible with water, 150

80

85

90

95

100

105

110

115

120

125

130

135

140

145

application should be made to the substantially dry web, but with a water miscible solvent application may be made either to the wet or substantially dry web, but preferably to the dry web in order to facilitate solvent recovery.

By the practice of my invention according to either of the two modifications described above, I produce paper filled with alkaline filler, which paper is substantially opaque or possesses a considerable degree of opacity and which is suitable for printing or other purposes, and which is similar in appearance to, and by cursory observation is difficult to distinguish from, ordinary clay-filled paper of the same grade. Such paper may be sized if desired or unsized, but possesses a special receptivity to printing ink. My paper is unlike and should not be confused with, papers saturated with oils or the like, and which are transparent or translucent, and in the claims the word "paper" is to be construed as being restricted to such papers as are not saturated with the pasty and/or liquid material specified.

As an illustrative example of the manufacture of sized paper by practicing my invention according to the first modification, I may use a furnish containing 1000 lbs. fibrous furnish, 250 lbs. alkaline filler, and 40 lbs. of the non-waxy material of pasty consistency, the same being in emulsion form, together with 40 lbs. of alum, the alum preferably being added at the dilute stage of the papermaking operation. As an illustrative example for the manufacture of a substantially unsized paper possessing a special receptivity to printing ink, I may substitute for the 40 lbs. of pasty material in the furnish above, 10 lbs. of non-waxy material of liquid consistency, the same being in emulsion form. Starch in an amount of 20 lbs. for example may be advantageously employed in either of the above 40 furnishes.

As an illustrative example of the manufacture of sized paper by practicing my invention according to the second modification I may apply to a paper web containing alkaline filler a 5 per cent. solution of the non-waxy material of pasty consistency, the same being dissolved in petroleum ether. As an illustrative example of the manufacture of a substantially unsized paper possessing a special receptivity to printing ink, I may apply to a paper web containing alkaline filler a 2 per cent. solution of non-waxy material of liquid consistency, said material being dissolved in petroleum ether. In either of the above cases the web may advantageously contain 55 starch.

It is to be understood that the above examples are to be taken as illustrative only and not as limiting, because, as will be apparent, I may carry out my invention with a wide variation as to materials, proportions, and conditions, and still obtain satisfactory results.

The word "solid" may be used to define two distinct characteristics of a substance. One characteristic is that which a substance possesses at any given temperature which makes it incapable, without the application of pressure, of spontaneously or quickly changing its shape, at least when a small bulk of the substance say 25 cubic centimeters is being considered. The second characteristic that may be defined by the term "solid" is that possessed by certain substances, of exhibiting substantial resistance to attempts at penetration.

Where I use the word "pasty" herein I mean that the substance so characterized possesses so-

lidity according to the first definition above but not according to the second. In other words, "pasty" substances are solid in that at ordinary or room temperature, when in small bulk, they will not exhibit flow or will exhibit it only with extreme slowness, but on the other hand are sufficiently soft so that the finger with only slight pressure will penetrate the mass in a manner in which it will not penetrate a waxy material such as fully refined paraffin for example.

Where I use the word "liquid" herein, I mean that a substance so characterized will exhibit flow at ordinary or room temperature.

As will be apparent there is actually an imperceptible gradation possible between the pasty and liquid condition, but the above definitions will distinguish between them with sufficient accuracy for commercial purposes.

The organic substantially water insoluble non-waxy materials substantially inert to alkaline 95 filler and of pasty and liquid consistency which are used in the practice of my invention may be derived from any available source. Examples are hydrocarbons which may be derived, for example, from petroleum, shale, lignite, earth wax, 100 or other natural or artificial source (whether animal, vegetable or mineral). Other examples are synthetic resinous products made, for example, by condensation. However, among those materials which I may use I do not intend to include such black or substantially black colored materials, which because of their color, are not feasible for use in white papers, or even in papers which are somewhat colored such as kraft or the like.

Where I use the word "liquid" herein in reference to non-waxy material or the like I mean to limit myself to liquids which do not have a vapor pressure sufficiently high spontaneously to evaporate to a substantial degree at ordinary or 110 room temperature, or at a temperature to which paper may be subjected in the manufacturing process subsequent to the inclusion of such liquid either in the mix or in the paper web, as obviously the inclusion of any low boiling liquid 115 would be of little or no avail owing to its substantial removal from the paper either spontaneously or by the heat to which the paper web containing such liquid was subjected.

In place of alum I may use other aluminum 125 salts or other metallic salts such as zinc sulphate or the like, or other acidic materials such as acid, sodium bisulphate or the like.

By the term "alkaline filler", I mean substantially water insoluble filler which when agitated 130 in contact with freshly boiled distilled water, say for an hour, will impart a pH value to such water greater than 7.0, that is, which will be on the alkaline side of the neutral point. Among fillers included in this group may be mentioned calcium 135 carbonate, of which lime mud from the causticizing process is one form; calcium carbonate magnesium basic carbonate employed in the paper disclosed in my United States Patent No. 1,595,-416, issued August 10, 1926; calcium carbonate 140 magnesium hydroxide disclosed in my United States Patent No. 1,415,391, issued May 9, 1932; and other substantially water insoluble normal or basic carbonates of alkaline earth metals (which expression is herein intended to include magnesium), or compounds, double salts, or physically associated mixtures of these with one or more other acid soluble materials of a substantially water insoluble nature.

By the term "alkaline filler", I also intend to include fibrous material and/or other material such as paper coating constituents or the like containing one or more compounds of the character referred to, such as "old papers" or similar papers, "broke" or the like.

When I use the word "paper" herein, I use it in the broad sense to include products of manufacture of all types and of all weights and thicknesses, which contain as an essential constituent a considerable amount of prepared fibre and which are capable of being produced on a Fourdrinier, cylinder, or other forming, felting, shaping or molding machine.

When I speak of paper as having a "special receptivity to printing ink" or "greater printing ink receptivity" or the like, I do not mean that said paper necessarily satisfies any one specific test such as rate of water or oil penetration or the like; but rather I mean broadly that, regardless of the result of any specific test performed on said paper, the paper so characterized possesses improved printing qualities.

The term "fibrous mix" or "paper mix" as used herein is intended to mean a mix of various constituents including fibre from which paper may be made either directly or after the addition of other ingredients.

While I have described in detail the preferred embodiment of my invention, it is to be understood that the details of procedure, the proportion and kinds of ingredients, and the arrangement of steps may be widely varied without departing from the spirit of my invention or the scope of the subjoined claims.

I claim:

1. Filled paper comprising fibrous material, alkaline filler, and at least one of a class of substantially water insoluble non-waxy organic materials substantially inert to alkaline filler comprising materials of pasty and liquid consistencies, in the absence of substantially water insoluble waxy organic material substantially inert to alkaline filler.

2. Filled paper comprising fibrous material, alkaline filler comprising calcium carbonate, and at least one of a class of substantially water insoluble non-waxy organic materials substantially inert to alkaline filler comprising materials of pasty and liquid consistencies, in the absence of substantially water insoluble waxy organic material substantially inert to alkaline filler.

3. Filled paper comprising fibrous material, alkaline filler comprising calcium carbonate and magnesium compound, and at least one of a class of substantially water insoluble non-waxy organic materials substantially inert to alkaline filler comprising materials of pasty and liquid consistencies, in the absence of substantially water insoluble waxy organic material substantially inert to alkaline filler.

4. Filled paper comprising fibrous material, alkaline filler, and substantially water insoluble non-waxy organic material of pasty consistency substantially inert to alkaline filler, in the absence of substantially water insoluble waxy organic material substantially inert to alkaline filler.

5. Filled paper comprising fibrous material, alkaline filler, and substantially water insoluble non-waxy organic material of liquid consistency substantially inert to alkaline filler, in the absence of substantially water insoluble waxy organic material substantially inert to alkaline filler.

6. Filled paper comprising fibrous material, al-

kaline filler, and non-waxy hydrocarbon of pasty consistency in the absence of waxy hydrocarbon.

7. Filled paper comprising fibrous material, alkaline filler, and non-waxy hydrocarbon of liquid consistency in the absence of waxy hydrocarbon. 80

8. Filled paper comprising fibrous material, alkaline filler, substantially water insoluble non-waxy organic material of pasty consistency substantially inert to alkaline filler, and size, in the absence of substantially water insoluble waxy organic material substantially inert to alkaline filler. 85

9. Filled paper comprising fibrous material, alkaline filler, substantially water insoluble non-waxy organic material of liquid consistency, and size, in the absence of substantially water insoluble waxy organic material substantially inert to alkaline filler. 90

10. Filled paper comprising fibrous material, alkaline filler, non-waxy hydrocarbon of pasty consistency, and size, in the absence of waxy hydrocarbon. 95

11. Filled paper comprising fibrous material, alkaline filler, non-waxy hydrocarbon of liquid consistency, and size, in the absence of waxy hydrocarbon. 100

12. Filled paper comprising fibrous material, alkaline filler, at least one of a class of substantially water insoluble non-waxy organic materials substantially inert to alkaline filler comprising materials of pasty and liquid consistencies, and precipitated size, in the absence of substantially water insoluble waxy organic material substantially inert to alkaline filler. 105

13. Filled paper comprising fibrous material, alkaline filler, at least one of a class of substantially water insoluble non-waxy organic materials substantially inert to alkaline filler comprising materials of pasty and liquid consistencies, and aluminum compound, in the absence of substantially water insoluble waxy organic material substantially inert to alkaline filler. 115

14. Filled paper comprising fibrous material, alkaline filler, at least one of a class of substantially water insoluble non-waxy organic materials substantially inert to alkaline filler comprising materials of pasty and liquid consistencies, and starch, in the absence of substantially water insoluble waxy organic material substantially inert to alkaline filler. 120

15. The steps in a process of manufacturing paper filled with alkaline filler, comprising mixing fibrous material, alkaline filler, and at least one of a class of substantially water insoluble non-waxy organic materials substantially inert to alkaline filler comprising materials of pasty and liquid consistencies, in the absence of substantially water insoluble waxy organic material substantially inert to alkaline filler, and running said mix off on a paper machine. 125

16. The steps in a process of manufacturing paper filled with alkaline filler, comprising mixing fibrous material, alkaline filler, at least one of a class of substantially water insoluble non-waxy organic materials substantially inert to alkaline filler comprising materials of pasty and liquid consistencies, and acidic material, in the absence of substantially water insoluble waxy organic material substantially inert to alkaline filler, and running said mix off on a paper machine. 130

17. The steps in a process of manufacturing paper filled with alkaline filler, comprising mixing fibrous material, alkaline filler, at least one 135

- of a class of substantially water insoluble non-waxy organic materials substantially inert to alkaline filler comprising materials of pasty and liquid consistencies, and alum, in the absence of 5 substantially water insoluble waxy organic material substantially inert to alkaline filler, and running said mix off on a paper machine.
18. The steps in a process of manufacturing paper filled with alkaline filler, comprising mixing fibrous material, alkaline filler, at least one 10 of a class of substantially water insoluble non-waxy organic materials substantially inert to alkaline filler comprising materials of pasty and liquid consistencies, and size, in the absence of 15 substantially water insoluble waxy organic material substantially inert to alkaline filler, and running said mix off on a paper machine.
19. The steps in a process of manufacturing paper filled with alkaline filler, comprising mixing 20 fibrous material, alkaline filler, at least one of a class of substantially water insoluble non-waxy organic materials substantially inert to alkaline filler comprising materials of pasty and liquid consistencies, size, and acidic material, in 25 the absence of substantially water insoluble waxy organic material substantially inert to alkaline filler, and running said mix off on a paper machine.
20. In a method of manufacturing paper filled 30 with alkaline filler wherein material is added to a paper mix under conditions favoring the minimizing of the time and/or intimacy of contact of the constituents of the mix, the step of adding to said paper mix at least one of a class of 35 substantially water insoluble non-waxy organic materials substantially inert to alkaline filler comprising materials of pasty and liquid consistencies, in the absence of substantially water insoluble waxy organic material substantially 40 inert to alkaline filler.
21. In a method of manufacturing paper filled with alkaline filler wherein material is added to a paper mix under conditions favoring the minimizing of the time and/or intimacy of contact 45 of the constituents of the mix, the step of adding to said paper mix at least one of a class of substantially water insoluble non-waxy organic materials of substantially inert to alkaline filler comprising materials of pasty and liquid consistencies, 50 and size, in the absence of substantially water insoluble waxy organic material substantially inert to alkaline filler.
22. In a method of manufacturing paper filled with alkaline filler wherein material is added to 55 a paper mix under conditions favoring the minimizing of the time and/or intimacy of contact of the constituents of the mix, the step of adding
- to said paper mix at least one of a class of substantially water insoluble non-waxy organic materials substantially inert to alkaline filler comprising materials of pasty and liquid consistencies, size, and acidic material, in the absence of 80 substantially water insoluble waxy organic material substantially inert to alkaline filler.
23. In a method of manufacturing paper filled with alkaline filler wherein material is added to a paper mix under conditions favoring the minimizing of the time and/or intimacy of contact of the constituents of the mix, the step of adding to said paper mix at least one of a class of substantially water insoluble non-waxy organic materials substantially inert to alkaline filler comprising materials of pasty and liquid consistencies, and precipitated size, in the absence of 85 substantially water insoluble waxy organic material substantially inert to alkaline filler.
24. In a method of manufacturing paper filled with alkaline filler wherein material is added to a paper mix under conditions favoring the minimizing of the time and/or intimacy of contact of the constituents of the mix, the step of adding to said paper mix at least one of a class of 90 substantially water insoluble non-waxy organic materials substantially inert to alkaline filler comprising materials of pasty and liquid consistencies, and acidic material, in the absence of substantially water insoluble waxy organic material substantially inert to alkaline filler.
25. In a method of manufacturing paper filled with alkaline filler wherein material is added to a paper mix under conditions favoring the minimizing of the time and/or intimacy of contact of the constituents of the mix, the step of adding to said paper mix at least one of a class of 95 substantially water insoluble non-waxy organic materials substantially inert to alkaline filler comprising materials of pasty and liquid consistencies, and acidic material, in the absence of substantially water insoluble waxy organic material substantially inert to alkaline filler.
26. In a method of manufacturing paper filled with alkaline filler wherein material is added to a paper mix under conditions favoring the minimizing of the time and/or intimacy of contact of the constituents of the mix, the step of adding to said paper mix at least one of a class of 100 substantially water insoluble non-waxy organic materials substantially inert to alkaline filler comprising materials of pasty and liquid consistencies, and acidic material, in the absence of substantially water insoluble waxy organic material substantially inert to alkaline filler.
- 105
- 110
- 115
- 120
- 125
- 130

HAROLD ROBERT RAFTON.

CERTIFICATE OF CORRECTION.

Patent No. 1,957,474.

May 8, 1934.

HAROLD ROBERT RAFTON.

It is hereby certified that error appears in the printed specification of the above numbered patent requiring correction as follows: Page 1, line 5, for "insolube" read insoluble; page 3, line 142, for "1932" read 1922; page 5, line 48, claim 21, strike out the word "of"; and line 49, for "consistences" read consistencies; and that the said Letters Patent should be read with these corrections therein that the same may conform to the record of the case in the Patent Office.

Signed and sealed this 24th day of July, A. D. 1934.

Bryan M. Battey

(Seal)

Acting Commissioner of Patents.